

## UNITED STATES PATENT OFFICE

SHINTA MATSUNAWA, FUSATOSHI NOZAWA, AND MASUHIRO SUZUKI, OF TOKYO, JAPAN,  
 ASSIGNORS TO KABUSHIKI KAISHA SUMITOMO SEIKOSHO, OF OSAKA, JAPAN, A  
 CORPORATION OF JAPAN

## HEAT-TREATMENT OF METALS

No Drawing. Application filed January 16, 1933, Serial No. 652,096, and in Japan February 5, 1932.

This invention relates to improvements in heat-treatment of metals wherein properly heated metals are quenched in a mixture of oil and water.

5 The chief object of this invention is to obtain a process whereby the final effect of the heat-treatment can be attained in a single step, that is, quenching only, while the hereto known heat-treatment of metals generally consists of two steps, that is, quenching and 10 tempering.

Another object of this invention is to obtain a liquid to be used for heat-treatment as the 15 cooling medium in which heated metals are quenched.

A further object of this invention is to obtain a cooling medium which can keep its emulsive condition without requiring any 20 subsequent agitation while heated metals are being quenched therein.

In the known heat-treatments of metals, properly heated metal is quenched in either water, oil or a mixture of water and oil, but the quenching effect is so violent that an 25 article fit for ready use can be scarcely obtained without subjecting the treated metal to a subsequent treatment called tempering. For instance, when a spring for vehicles made of carbon-steel plates or rod is quenched 30 in either water, oil or the mixture, the micro-structure obtained is martensite or the like, and unfit for a spring. Therefore the spring has to be subjected to re-heating at a tempering temperature of 400° C.-500° C. in 35 order to moderate the violent effect of the quenching, whereby the proper strength and toughness of the spring are obtained.

When the mixture of water and oil is used, it is required to be continuously stirred while 40 the article is being quenched therein because the two substances are ready to separate from each other. Moreover, water, when mixed with oil, takes the form of comparatively large particles, and large vapour bubbles are 45 formed when the particles touch the highly heated surface of metal, resulting in an uneven effect of heat-treatment, which often causes cracks in the material. These drawbacks can be removed by this invention.

50 The main feature of this invented process

lies in the fact that a single heat treatment is generally sufficient for the purpose, fully utilizing the effect of the treatment in accordance with the kinds and uses of the material, and homogeneous substance can be obtained 55 without the least danger of spoiling the article. The process can be applied on a large scale as well as a small scale with the same results.

According to this invention, a mixture of 60 water and oil is used as the cooling medium in heat-treatment, but the oil to be used for this purpose is limited to mineral oil such as machine-oil, cylinder oil or heavy oil as mixed with petrolene of from 0.5% to 10%, 65 which has been extracted from petroleum-pitch with a solvent such as benzine or tetrachloride of carbon. The quantity of water to be mixed with oil is determined in accordance with the kind and use of the metal, and 70 the mixture should be sufficiently agitated until it makes an emulsion.

When this cooling medium is used for heat treatment, the violent effect by water is moderated by the addition of oil, and as 75 the water particles are very fine and are evenly distributed in the medium, the vapour bubbles which may be produced on the surface of the heated metal are very small, and the effect of heat treatment is uniform over the 80 whole surface, so that thermal strain in the article is minimized, and springs can obtain properly balanced rigidity, tenacity and toughness and tools a superior cutting quality.

The main characteristic of this invention is that the cooling medium keeps its emulsive condition for a long time requiring no subsequent agitation after it has been once emulsified. This is due to the use of mineral oil as 90 mixed with petrolene from 0.5% to 10%. Since no agitating apparatus such as pumps or propellers is required, the process can be applied with the same result on a large scale 95 as well as a small one.

The invention may be further explained by way of the following examples.

1. A spring for vehicles made of spring steel plates or rod containing carbon of 0.6 to 0.88% is heated up to 800° C.-830° C., and 100

is quenched in a cooling medium at a temperature of 40° C., the composition of the medium being 20% of water and 80% of machine oil containing 3% petrolene, emulsified by 5 means of a colloid-mill. With only one quenching, a good spring of troostic-sorbite structure having 47-53 (Shore hardness) is obtained.

2. A bit made of high-speed tool-steel containing 0.9% carbon, 20.3% tungsten and some percentage of cobalt and chromium is heated up to 1350° C., and is quenched in an emulsified cooling medium at the temperature of 40° C., the composition of the medium 10 being 80% of water and 70% of machine oil containing 5% petrolene. The bit thus obtained can easily cut a high-manganese rail steel which contains 14.0% manganese and 1.0% carbon, and has been quenched in water 15 from the temperature of 1050° C. forming 20 austenite structure.

By this process not only fuel and labour can be saved, but thermo-cracking and loss of material can be avoided, which may be caused by repeated heating.

What we claim is:—

1. A process of heat treatment of metals, comprising quenching the heated metals in a cooling medium, comprising an emulsion of water and a mineral oil containing 0.5% to 75 10% petrolene.

2. A quenching medium for the heat treatment of metal, comprising an emulsion of water and a mineral oil containing 0.5% to 10% petrolene.

In testimony whereof we affix our signatures.

SHINTA MATSUNAWA.  
FUSATOSHI NOZAWA.  
MASUHIRO SUZUKI.